

May 19, 1936.

R. L. LEVENTRY

2,041,612

METALLURGICAL FURNACE

Filed June 3, 1933

2 Sheets-Sheet 1



Inventor

Roy L. LEVENTRY.

*Rickey & Watt*  
Attorney

May 19, 1936.

R. L. LEVENTRY

2,041,612

## METALLURGICAL FURNACE

Filed June 3, 1933

2 Sheets-Sheet 2



## Inventor

ROY L. LEVENTRY.

*Rickey & Hatt*  
Attorney

## UNITED STATES PATENT OFFICE

2,041,612

## METALLURGICAL FURNACE

Roy L. Leventry, Youngstown, Ohio, assignor to  
The Republic Steel Corporation, Youngstown,  
Ohio, a corporation of New Jersey

Application June 3, 1933, Serial No. 674,250

4 Claims. (Cl. 266—43)

This invention relates to improvements in metallurgical furnaces and more particularly metallurgical furnaces of the open-hearth type. The general nature and operation of open-hearth steel furnaces are well understood in the art. The most widely used furnace of this character is the one which is known as the basic open-hearth furnace. In these furnaces the charge i. e. the metal in process of treatment, is subjected to the action of radiated heat, the flame necessary for this purpose being produced by the combustion of streams of combustible gas and air. It is customary in such furnaces to have them provided with a chimney draft sufficient to catch the flame about in the middle of the laboratory and drag it out through the ports on the opposite side from which it entered without allowing it either to drop down and touch the bath or to impinge upon the roof, and the draft has also to do the work of overcoming the friction of the outgoing regenerators and flues, such regenerators and flues being provided as a means for assuring that the entering air and combustion gases, when subsequently allowed to flow through such regenerators and flues, on entering the laboratory, will have the requisite temperature. It is obvious that under the stated requirements the draft through such a furnace during its operation is very considerable. The gas and air are given a velocity which causes them to enter the furnace with some force and the construction of the ports directs the streams in the desired manner. In passing through the laboratory the gas should be spread out all over the width of the hearth beneath the air as the latter must be kept away from direct contact with the bath. The products of combustion of the flame together with any materials which may have been picked up in passing through the furnace are drawn along the furnace walls and into the exit flues with considerable power. It is well known that during the operation of the furnace particles of slag, dust, and dirt are carried over with the outgoing gases and because of this the so-called slag pockets or dirt pockets are ordinarily provided as a part of the structure of such furnaces. In spite of the presence of such slag pockets, however, the space between the bricks of the checker-work of the regenerators becomes partially choked, and for this reason, as well as because the deposit of the slag, dust, and dirt particles makes the surface of the bricks rough, the total area between the bricks must be much larger than the area of the ports, so that the

velocity of the gas will not be lessened. These conditions indicate that there is a very considerable amount of foreign material picked up and carried along by the high velocity of the gas streams passing through the laboratory.

In the construction of open-hearth furnaces it has been customary to use magnesite as a lining for the bottom of the furnace as it is well resistant to basic slag which contains iron oxide, silica dioxide and lime but the topmost layer or working bottom and the repairs put in during the intervals of the furnace life, are usually made of dolomite. The sides and roof of the furnace are generally made of silica bricks.

Magnesite is the most expensive of the several materials made use of in the construction of an open-hearth furnace and a cheaper equally good substitute material has long been sought for. Substances such as chromite and dolomite have been tried but have not been found the equal of burnt magnesite although dolomite has proved itself to be a very desirable material for use as a patching substance in filling up the holes made in the magnesite during the operation of the furnace. Several years ago a suggestion was made to the effect that olivine rock, inasmuch as it possessed properties enabling large pieces or blocks of the rock to be heated to very high temperatures while retaining its mechanical strength at high temperatures, might be available in the construction of metallurgical furnaces to replace magnesite. Experiments were made with olivine but they proved to be failures with the result that the use of olivine as a lining material for open-hearth furnaces was discarded and discredited.

I have now discovered that the cause for the failure of olivine in metallurgical furnaces is to be found chiefly in its incapacity to resist the effect of the action of lime. In the presence of lime such as exists in the molten metal bath as the result of the addition of dolomite patching material olivine disintegrates. This disintegrating effect is most active in those regions where most lime exists, i. e. at or near the immediate vicinity of the slag line. Accordingly, inasmuch as the slag is itself in contact with the lining of the bottom of the furnace and is also subjected at its surface to the vigorous sweeping action of the gas currents passing through the furnace and in their passage vigorously affecting the walls of the furnace and the exhaust orifices and ducts, olivine was regarded as a peculiarly inappropriate material to be used at any point in the structure

of a metallurgical furnace of the open-hearth type.

I have now discovered, however, that there is a difference in the effect on olivine as between contact with lime-bearing substances in a bath and contact with lime-bearing substances or particles such as may be swept from the surface slag of such a bath against olivine by the type of draft which is characteristic of an open-hearth furnace operation. In the former case the olivine is useless while in the latter the olivine, instead of disintegrating, appears to become stronger and more highly refractory. Thus, although olivine does not resist the basic slag in the bath, it does well resist the effect of iron oxide and silica dioxide while such lime or lime-bearing substances as may be physically carried into contact with olivine by a flame of such fierce velocity and constitution as passes through a basic open-hearth furnace seems to be ineffective on the olivine.

Based on these foregoing discoveries, it occurred to me that beneficial effects might result if, instead of attempting to use olivine as a material to replace the magnesite lining of the bottom 25 of the furnace, it were used at least partially to replace or to form a surfacing layer for the silica bricks used for the sides of the open-hearth furnace. Iron oxide is very active on silica brick and tends to slag it, while, as above stated, olivine 30 resists the action of iron oxide. Even the most refractory silica bricks can be melted by the intense heat of the direct impact of the flame. The silica brick walls constituting the side walls of an open-hearth furnace are usually thin, which results in great radiation of heat from the furnace chamber but as one authority puts it "This has to be endured, as thicker walls produce endless trouble by expansion and contraction".

Based on the foregoing considerations and in order to put my discovery to practical use I designed a basic open-hearth furnace in which, although the bottom was lined as usual with magnesite, patchable and repairable at will by the introduction of dolomite, the end walls, at 45 least at those parts thereof which are affected by the impingement of the gas flow, and those portions of the front and rear walls of the furnace which were above the slag line and within the region affected by the flame and the gas draft 50 were constituted of olivine. Furnaces of this design were put into practice and use and found to constitute a material improvement over furnaces of like nature constructed in accordance with the fundamentals of practice theretofore followed. 55 The term olivine applies to a mineral of varying degrees of constitution, not every one of which can be satisfactorily employed for the purposes under consideration.

I have however found that certain grades of olivine, which occur in extensive deposits in the United States and which are therefore relatively cheap and readily obtainable, may be used satisfactorily for lining parts of metallurgical furnaces and will satisfy the requirements.

Olivine is an anhydrous silicate of magnesium and iron. Altho the composition varies somewhat, a formula which may be considered more or less typical is  $(\text{MgFe})_2\text{SiO}_4$ . An average theoretical composition of olivine may include about 48% of  $\text{MgO}$ , 42% of  $\text{SiO}_2$  and 10% of iron calculated as  $\text{FeO}$ . The iron content ranges from a low amount such as 2% or 3% to as high as about 20% in different forms of olivine.

Olivine containing between about 4% and

about 15% of iron, calculated as  $\text{FeO}$ , may be used satisfactorily as a lining material for metallurgical furnaces when arranged as hereinabove set forth. Another way of describing the composition of olivine within the preferred range, is 5 on the basis of the ratio of magnesium to iron. This ratio varies in different types of olivine from as low as 2 to 1 to as high as 16 to 1. I prefer a ratio of not less than 3 to 1 and not more than about 8 to 1, and more especially prefer a ratio 10 of between 5 to 1 and 8 to 1. As a result of extended tests and experiments in actual use, I have found that olivine within the foregoing composition range and conditions of use above specified has been entirely satisfactory and is favorably comparable with the more expensive and high grade furnace lining materials, such as chrome ore. 15

A preferred olivine for the foregoing uses contains between about 7% and about 10% of iron, 20 calculated as  $\text{FeO}$ .

When olivine of the foregoing composition range is used as a lining material for walls which are within the gas flow region but above the slag line, it is satisfactory as a lining material. Ordinarily lime reacts with it to lower its fusion temperature but I believe that the high temperatures and oxidizing atmospheres to which olivine is subjected in the regions of high velocity 25 gas flow combine notwithstanding the fact that the rapidly moving gas has the opportunity of picking up or carrying along with it lime-containing particles from the slag, to bring about a partial sintering and an oxidation of the iron content from a ferrous to a ferric state, thereby 30 rendering olivine of the foregoing composition highly refractory when used and positioned in the described manner and places. Moreover, I believe that such high temperatures and highly 35 oxidizing atmospheres tend to produce a bond 40 between contacting pieces of olivine. At any rate, such olivine when highly heated in the oxidizing atmosphere of an open hearth furnace, becomes stronger and more highly refractory and endures 45 long continued use. Such olivine stands up well under high furnace temperatures, has good load carrying strength, is not materially eroded even after many heats of steel have been made in a furnace lined above the slag line with it, and 50 the contacting pieces are, after some time, actually "glued" or fitted together and thus bonded to each other. Olivine within the stated composition range may be used as a lining material either in the form of suitably shaped blocks or in 55 the form of lumps of different sizes, made up with any suitable binding material such as ground chrome ore.

Reference may be had to the accompanying drawings which illustrate the applicability of 60 my invention to a conventional open hearth furnace and wherein similar reference characters denote corresponding parts and wherein:

Fig. 1 is a horizontal sectional view taken on a plane through the mid portion of an open hearth 65 furnace.

Fig. 2 is a vertical section taken on line 2--2 of Fig. 1.

Referring to the drawings there is illustrated a conventional open hearth furnace having certain 70 portions thereof constructed of a refractory made in accordance with my invention. The open hearth furnace shown generally at 1 includes a foundation grillage indicated at 2, having transverse members 2' to which are secured at their 75

lower ends, vertically extending buckstays 3, and rear buckstays 3'. The rear buckstays 3' are located opposite front buckstays 3 and the opposite buckstays are connected together at their 5 upper ends by tie rods 4.

Each of the rear buckstays 3', however, includes a substantially vertically extending lower strut 5 and a substantially vertical upper strut 6, outwardly offset from the lower strut and being connected at its lower end with the upper end of the lower strut by a substantially horizontal ledge supporting beam 8. A diagonal brace 9 is provided for connecting the outer end of the beam 8 with the lower end of the strut 5. Within the 10 structural frame work thus formed the refractory materials of the furnace are supported which includes a furnace bottom 10 preferably made of conventional refractory brick and a vertically extending refractory brick front wall 11, abutting 15 the buckstays 3.

Opposite the front wall and abutting the lower vertical strut 5 of the buckstays 3' is provided a vertically extending brick wall 12. The brick walls 11 and 12 are made of any suitable refractory such as silica brick now in common use. These walls made of silica brick extend upwardly as far as the slag line which is designated as 25 at 13. Suitable vertical extensions 14 and 15 of the front and rear walls 11 and 12 respectively 30 are provided. These extensions are connected by roof 16 of any usual construction. The walls 14 and 15 being disposed above the slag line are constructed of a refractory olivine material.

Furnace ends 16 and 17 may be provided of 35 any usual construction and include the air ports 19 and 20 and a gas port 21. The walls defining these ports being out of contact with the slag disposed on the bath disposed in the furnace are constructed of olivine refractory.

Having thus described my invention so that those skilled in the art may practice the same, what I desire to secure by Letters Patent is defined in what is claimed.

What is claimed is:

1. An open-hearth steel furnace, the lining whereof is subjected at high temperatures to the effects of a basic slag, said furnace comprising a bottom adapted to support a molten metallic bath, a hearth lining for said bottom composed of refractory material capable of withstanding the action of a basic slag, said lining covering the bottom of said furnace and extending up the walls thereof to a point above the line where the slag on the bath contacts with said lining, and a lining for portions of the walls of said furnace arranged to form contact surfaces

for the hot gases passing through the furnace, said last mentioned lining being composed of olivine containing approximately from 4 to 15% of iron calculated as FeO and being resistant to the hot gases passing at high velocity through the furnace and over the slag of the bath and laden with foreign material picked up in the furnace. 5

2. In a basic open hearth steel furnace where the lining thereof is subjected at high temperatures to the effects of a basic slag containing appreciable amounts of lime, a lower lining composed of basic refractory material capable of withstanding the action of a basic slag, said lining covering the bottom of said furnace and 10 extending up the walls thereof to a point above where the slag on the bath will contact with the lining of the furnace, and an upper lining covering upper portions of the walls of said furnace and being in contact with the hot gases passing 15 through the furnace, said upper lining being composed of olivine containing approximately from 4 to 15% of iron calculated as FeO, the contacting pieces of which have been formed into bonded and partially sintered masses at the high heat 20 in the oxidizing atmosphere and are resistant to the hot gases passing at high velocity through the furnace and over the slag of the bath and laden with foreign material picked up in the furnace. 25

3. In a basic open hearth steel furnace, a lining comprising basic-slag-resisting refractory material for the bottom and lower side walls up to a point slightly above the slag line, and a lining for the upper side walls in contact with the hot gases extending from the lower walls to the roof of the furnace, said lining for the upper side walls consisting of olivine containing between about 4% and about 15% of iron calculated as FeO and being resistant to the hot gases passing at high 30 velocity through the furnace and over the slag of the bath and laden with foreign material picked up in the furnace. 35

4. In a basic open hearth steel furnace, a lining comprising basic-slag-resisting refractory material for the bottom and lower side walls up to a point slightly above the slag line, and a lining for the upper side walls in contact with the hot gases extending from the lower walls to the roof of the furnace, said lining for the upper side walls consisting of olivine containing about 10% iron calculated as FeO and being resistant to the hot gases passing at high velocity through the furnace and over the slag of the bath and laden with foreign material picked up in the furnace. 40 45 50 55

ROY L. LEVENTRY.